

# United States Patent Office.

WILLIAM H. MOSS, OF NEW RICHMOND, OHIO.

*Letters Patent No. 80,559, dated August 4, 1868.*

## IMPROVED OIL FOR WOOL.

The Schedule referred to in these Letters Patent and making part of the same.

TO ALL WHOM IT MAY CONCERN:

Be it known that I, WILLIAM H. MOSS, of the village of New Richmond, in the county of Clermont, and State of Ohio, have invented a new and useful Compound Oil for the Purpose of Greasing Wool in the manufacture of woollen goods, and for use in carding and spinning wool; and I do hereby declare the following to be a full, clear, and exact description thereof.

This compound oil is composed of the following ingredients in the following-stated proportions, to wit: Twenty-five pounds of unslaked lime, twenty gallons of water, twenty gallons of lard-oil.

The process of mixture is as follows, to wit: The twenty-five pounds of unslaked lime are placed in a barrel or other vessel that will answer the purpose, and the twenty gallons of water are then added. The whole is then well stirred together and thoroughly mixed. It then is left to stand twelve hours without being stirred or shaken, when the clear liquor is drawn off and the twenty gallons of lard-oil added, and the compound oil is ready for use, all of which ingredients are necessary to its manufacture.

This compound oil can be made by manufacturers of woollen goods at nearly one-half the cost of lard-oil, and is much more efficient for the purpose of greasing wool, and in carding and spinning the same, than pure lard-oil or any other oil now known.

The lime in this compound is calcareous in its nature, and when mixed with the water and oil, as above set forth, it becomes of the nature of alkali, and so, in fulling and scouring wool, it is cleaned much easier than any other oil, and at a saving of one-third of the soap required for other oils, and one-third the actual time and labor, making a clear saving to the manufacturer, in all, of two-thirds or three-fourths more than any other oil or oils now known, time, labor, and materials included.

This compound oil being thoroughly tested against pure lard-oil (the very best known) in greasing and carding and spinning wool, it was found, on every trial, that the wool greased, carded, and spun by and with the use and help of this compound oil was far easier to cleanse, as before stated; it took colors more readily, brighter, and more perfectly than a similar amount of wool greased, carded, and spun by and with the help of a like quantity of pure lard-oil.

What I now claim as my own invention, and desire to secure by Letters Patent, is—

The preparation of a compound oil, composed of the ingredients and in the proportions, and made in the way and manner, substantially as set forth above, for application to the use and manufacture of all kinds of woollen goods, and the greasing, carding, cleansing, and spinning of all kinds of wool.

Witnesses:

FRANK DAVIS,  
JOHN W. LENNIN.

WILLIAM H. MOSS.